

# United States Patent

[11] 3,619,122

[72] Inventor **Anthony De Maria**  
Easton, Pa.  
[21] Appl. No. **787,204**  
[22] Filed **Dec. 26, 1968**  
[45] Patented **Nov. 9, 1971**  
[73] Assignee **GAF Corporation**  
New York, N.Y.

[54] **PROCESS FOR DYEING POLYAMIDE FIBERS**  
6 Claims, No Drawings

[52] U.S. Cl..... **8/173,**  
8/178  
[51] Int. Cl..... **D06p 5/04**  
[50] Field of Search..... **8/173, 178,**  
**89; 260/481**

[56] **References Cited**

UNITED STATES PATENTS

2,028,091 1/1936 Jaeger ..... 260/481  
2,176,423 10/1939 Jaeger ..... 260/481  
2,558,733 7/1951 Cresswell et al. ..... 8/177

FOREIGN PATENTS

802,574 10/1958 Great Britain ..... 8/65

Primary Examiner—George F. Lesmes  
Assistant Examiner—T. J. Herbert, Jr.  
Attorneys—Walter C. Kihm and Samson B. Leavitt

**ABSTRACT:** A process for producing barre free dyeing of polyamide fibers comprising dyeing said fibers with a composition comprising an acid dye and a dialkyl sulfosuccinate having the following formula:



wherein R is an alkyl radical having from four to 18 carbon atoms and M is either an alkali metal, alkaline earth metal, ammonium, or a substituted ammonium radical.

## PROCESS FOR DYEING POLYAMIDE FIBERS

The instant invention is directed to a process of uniformly dyeing polyamide fibers.

In the past the commercial practice of dyeing the synthetic linear polycarbonamides more familiarly known as nylon has been carried out by means of dispersed or acetate dyestuffs. These dispersed dyestuffs have great covering power for nylon yarns and are not highly sensitive to the normal variations found in such yarns. However, the dispersed or acetate colors lack fastness to light and to washing. In contrast, the anionic dyestuffs best exemplified by the class of acid dyes have extremely good fastness on nylon to both light and washing. It has not been commercially feasible to utilize the anionic dyestuffs in the majority of nylon filament dyeings, however, since those dyestuffs are extremely sensitive to variations between different fibers and different parts of the same fibers. Nylon yarns which have been spun at different times or from different lots of polymer demonstrate these variations most clearly. Frequently yarns spun at different times are dyed to different shades with the anionic dyestuffs when dyed by standard dyeing procedures. As a result the nylon fabrics dyed with anionic dyes are often colored in an uneven fashion, showing streaks and shade depth variations in knitted goods, and barré effects, warp streaks and the like inwoven goods. The inability to secure even dyeing of nylon yarns and fabrics is believed to be due to slight variations in the physical structure of the parent polymers such as variations in orientation due to the drawing to which each filament is subjected. Other factors occurring in the spinning and processing of the yarn, the mechanical action of the textile machinery used in the knitting or weaving of the fabrics, and perhaps other causes as well, also affect the even dyeing of nylon yarns and fabrics. This inability to evenly dye nylon yarns and fabrics with the anionic dyestuffs has curtailed the large scale use of such dyestuffs for dyeing the nylon materials on which they exhibit excellent light and wash fastness properties.

In addition, many explanations have been offered to explain the barré phenomenon, none of which has been completely satisfactory. However, it is known that both the drawing of the polymer filament and the heat history of the filament itself are responsible for the apparent lack of uniformity in the final dyeing. The drawing of the polymer filament is a necessary step to the full development of the desirable physical properties of the fiber, such as strength and elasticity. During the drawing the polymer molecules become highly oriented, therefore creating the possibility and conditions for the formation of groups of chain ends alternating with or following highly crystalline areas of packed parallel molecules. Since it has been theorized that the terminal amino groups of the polymer chains are the more important and more readily accessible sites to the dye, it is easily seen why the uniformity of dyeing would be impaired by the drawing of the polymer filament.

With regard to the heat history of the filament, it can be said that heat affects the polymer structure of the filament at each processing step. Exposure to heat results in an increase in the crystallinity of the polymer along with additional molecular rearrangement phenomena such as chain dislocation etc. The extent of these changes is influenced by the temperature reached and by the moisture present.

Numerous dyeing systems have been developed in an attempt to overcome the lack of levelness and uniformity associated with the use of acid dyes. These systems have included cationic agents which tend to complex the acid dye and release it gradually so as to retard the dyestuff strike, and the use of colorless anions designed to compete with the dye for the fiber dye sites so as to retard the dyestuff.

All of these systems, however, are suited to only a small number of dyes and become limited by their own selectivity in this respect.

Therefore, it is an object of the instant invention to provide a dyeing system for polycarbonamides which produces a level, uniform, and barré free dyeing effect and which employs a large number of different dyestuffs.

Yet a further object of the instant invention is to provide a dyeing system which produces a barré free dyeing effect on polycarbonamides, said system comprising a sulfonated dialkyl succinic acid and an acid dyestuff.

As used in the instant specification the term "levelness" is meant to refer to a dyeing, the results of which are an evenly dyed appearance of a fabric or yarn. Poor levelness shows up in streaks or areas of light and dark color which have been unevenly dyed. This can be attributed to sharp variations in the temperature of the dye bath, too fast a rate of temperature increase, or other mechanical interferences such as poor agitation or uneven distribution of the fabric in the dye bath. The term "barré" is meant to refer to defective dyeing uniformity, caused, as we have previously discussed, by both the drawing of the polymer filament and the heat history of the filament itself. Therefore, while levelness is caused by factors affecting the process of dyeing, the potential for barré defects is inherent in the fiber.

With the instant invention, polycarbonamides are dyed with a level, barré free effect with a dialkyl sulfosuccinate salt and an acid dye. The useful sulfonated dialkyl succinate salts include those salts with from 12 to 40 carbon atoms such as:

bis(butyl) sulfosuccinate  
bis(ethyl) sulfosuccinate [bis(pentyl) sulfosuccinate]  
bis(hexyl) sulfosuccinate  
bis(heptyl) sulfosuccinate  
bis(octyl) sulfosuccinate  
bis(nonyl) sulfosuccinate  
bis(decyl) sulfosuccinate  
bis(undecyl) sulfosuccinate  
bis(dodecyl) sulfosuccinate  
bis(tridecyl) sulfosuccinate  
bis(tetradecyl) sulfosuccinate  
bis(pentadecyl) sulfosuccinate  
bis(hexadecyl) sulfosuccinate  
bis(heptadecyl) sulfosuccinate  
bis(octadecyl) sulfosuccinate

More particularly, these salts include but are not limited to alkali metal, i.e., lithium, potassium, sodium, alkaline earth metal, ammonium and substituted ammonium, salts, or any other water soluble salts of dialkyl sulfosuccinates.

bis(1,2-dimethyl-hexyl) sulfosuccinate  
bis(2,6-dimethyl-heptyl-4) sulfosuccinate  
bis(1,4-dimethyl-heptyl-4) sulfosuccinate  
bis(1,4-dimethyl-heptyl-3) sulfosuccinate  
bis(1,4-diethyl-heptyl) sulfosuccinate  
bis(1,3-diisopropyl butyl) sulfosuccinate  
bis(3,5-dimethyl-octyl-5) sulfosuccinate  
bis(1,7-diethyl tetradecyl-10) sulfosuccinate  
bis(1,3-dimethyl butyl-1) sulfosuccinate  
bis(3,8-dibutyl heptyl-5) sulfosuccinate  
bis(1,7-diphenyl octyl-4) sulfosuccinate, etc.

The above dialkyl sulfosuccinates are all old and well-known in the art. They may be prepared according to the methods disclosed in U.S. Patents 2,028,091 and 2,175,423 or by any other conventional method. These compounds generally correspond to the following formula:



wherein R represents an alkyl radical having from four to 18 carbon atoms, and M represents either an alkali metal, alkaline earth metal, ammonium, or substituted ammonium radical.

The sulfonated dialkyl succinates assist in producing level, barré free dyeings when they are employed at the beginning of the dye cycle in amounts of from 0.1 percent to 10 percent and preferably in amounts of from 0.1 to 6 percent. The percentages are based on the weight of the goods or fibers to be dyed. The amounts required are higher for lighter shades as a lower percentage of dye is employed and lower for darker

shades in which higher percentages of dyes are employed. Therefore, in general when one employs from 0.05 percent to 1 percent (OWF) of dye, said amounts based on the weight of the goods, one would use about 4 percent (OWF) of the sulfosuccinate. When 1 percent to 2 percent (OWF) of dye is employed, one would use about 2 percent (OWF) of the succinate, and about 1 percent (OWF) of the succinate would be employed when about 2-4 percent (OWF) of the dye is employed. The sulfonated dialkyl succinates can also be added at various stages during the dyeing process or they may be used to repair defective dyeings. The useful sulfonated dialkyl succinates have a retarding action on the dyestuff exhaustion and definitely affect mobility of the dye by increasing its migration and transfer properties.

The useful acid and direct dyes which may be employed in connection with the instant invention include water-soluble nonmetallized acid dyes of various groups such as monoazo, diazo, anthraquinone, etc. These dyes are preferably non-metallized complex containing acid dyes and include, but are not limited to

| C.I. Name                 | C.I. Number      |
|---------------------------|------------------|
| Milling Yellow O          | Acid Yellow 38   |
| Supranol Yellow GGA       | Acid Yellow 40   |
| Fast Light Yellow GGXN    | Acid Yellow 17   |
| Wool Fast Orange GA       | Mordant Orange 6 |
| Supranol Orange RA        | Acid Orange 45   |
| Supranol Red RL           | Acid Red 99      |
| Supranol Red PG           | Acid Red 85      |
| Supranol Brilliant Red BA | Acid Red 133     |
| Supranol Red PBX          | Acid Red 114     |
| Alizarine Supra Blue A    | Acid Blue 25     |
| Phenamine Scarlet B       | Direct Red 37    |
| Chrysophenine Y           | Direct Yellow 12 |
| Supra Light Rubine BLA    | Acid Red 32      |
| Alizarine Astrol B        | Acid Blue 27     |
| Alizarine Sky Blue BS     | Acid Blue 78     |
| Alizarine Supra Sky RA    | Acid Blue 62     |
| Alizarine Cyanine         |                  |
| Green GHN                 | Acid Green 25    |
| Alizarine Cyanine         |                  |
| Green GWA                 | Acid Green 44    |
| Sulphon Cyanine 5RA       | Acid Blue 113    |
| Sulphon Cyanine GRA       | Acid Blue 120    |
| Sulphon Cyanine GA        | Acid Blue 118    |
| Anthraquinone Violet D    | Acid Violet 34   |
| Alizarine Fast Gray BLN   | Acid Black 48    |
|                           | 61570            |
|                           | 61590            |
|                           | 26360            |
|                           | 26400            |
|                           | 26410            |
|                           | 61710            |
|                           | 65005            |

The dye system of the instant invention is operable at a broad range of pH's with the preferred range being a pH of from 3 to 7. Furthermore, the system may be employed at various temperatures and satisfactory dyeings are obtained even below the boil. The preferred temperature range, however, is from about 160° to about 230° F. In this regard, it is of note that when one employs the novel process of the instant invention, one is able to carry out dyeing procedures at lower temperatures than those conventionally employed in such processes.

In addition to the production of level and barre free dyeings in the coloring of other types of nylon materials, the instant system is also useful in connection with the dyeing of nylon carpetings. In the past, when nylon carpetings having a jute backing were dyed, the nylon became stained as a result of the natural coloring matter bleeding off the jute in the dye bath. Its concentration in the dye bath increases as the dyeing progresses, and the nylon which has a pronounced affinity for this brown-colored matter picks it up readily. The resulting brown coloration which has a very low-light fastness, adversely affects the fastness and the purity of the final shade. The use of dialkyl sulfosuccinates in the dyeing of jute-backed nylon carpets prevents the brown matter coming off the jute backing from affecting the final shade of the nylon surface.

In addition, it has also been found that the useful dialkyl sulfosuccinates can be employed to repair barre dyeings. These

sulfosuccinates as noted previously increase the migrating, the mobility and transfer properties of acid nonmetallized dyes. In general, the goods can be heated in a bath with the dialkyl sulfosuccinate to about 90°-120° F. An alkaline pH is established so as to encourage the migration of the dye off the fiber. Any suitable alkaline material may be employed such as ammonium hydroxide. The bath can be taken to the boil or close thereto over about 30 minutes and maintained there for at least about 45 minutes. At this point, a great deal of dye has been transferred from the fabric to the dye bath. To return this dye to the fiber in the presence of the barre suppressant which we have in the bath, a gradual addition of prediluted acetic acid can be made (about 2 percent OWF.) to bring about satisfactory exhaustion of the dye bath. The resulting dyeing, assuming that suitable dyestuffs have been used, should be barre free. If additional dyestuff is required for shade adjustment, it may be added at any time before the acetic acid additions.

The novel process of the instant invention can be employed in connection with numerous forms of polycarbonamide fibers, including but not limited to woven, felted, filament, staple fiber, yarn, slubbing, wound packages, etc.

The present invention will now be described by reference to the following specific examples. Such examples are presented for purposes of illustration only, and the present invention is in no way to be deemed as limited thereto.

#### EXAMPLE I

30 Comparative dyeings were made of 10 gram samples of textured nylon 66 (Banlon, Joseph Bancroft & Company) using dye baths comprising:  
 A. 0.2 percent OWF Dye plug 1 percent ethoxylated nonionic surfactant comprising nonyl phenol+30 mols E.O.,  
 35 75 percent active and 6 percent ammonium sulfate. (E.O. means ethylene oxide.)  
 B. 0.2 percent OWF Dye plus 4 percent Sodium bis-(2,6-dimethyl-heptyl-4)sulfosuccinate.  
 The baths were established at a ratio of 1 gram of fabric to 40 ccs. liquid, and the temperature raised to the boil over a period of 45 minutes, after the first 30 minutes of which 1 percent acetic acid (56 percent) was added to the bath (A). The dye baths were maintained at this temperature for a period of 1 hour, and the samples were subsequently rinsed and dried.  
 45 They were also critically examined for levelness and barre. The dyeings were tested for light fastness according to the AATCC Standard Method 16A-1964. A rating scale of 1 to 5 was used in which 5 indicates a level or barre free dyeing and 1 a dyeing showing an unlevelness or a pronounced degree of barre.

50 As may be seen from table I, there was a dramatic improvement in both levelness and barre effect when sodium bis-(2,6-dimethyl-heptyl-4)sulfosuccinate was employed in the dye bath.

TABLE I

| 60 | Employing dye bath                                  | Improvement in— |     |       |     |               |   |
|----|-----------------------------------------------------|-----------------|-----|-------|-----|---------------|---|
|    |                                                     | Levelness       |     | Barre |     | Lightfastness |   |
|    |                                                     | A               | B   | A     | B   | A             | B |
| 65 | Milling Yellow O (Acid Yellow 38—C.I. 25135)        | 2               | 5   | 2     | 4-5 | 6             | 6 |
|    | Supranol Yellow GGA (Acid Yellow 40—C.I. 18950)     | 4               | 5   | 4-5   | 4-5 | 3-4           | 5 |
|    | Fast Light Yellow GGXN (Acid Yellow 17—C.I. 18965)  | 4               | 4   | 3-4   | 4   | 4             | 4 |
|    | Wool Fast Orange GA (Mordant Orange 6—C.I. 26520)   | 4               | 4   | 3-4   | 4-5 | 6             | 6 |
|    | Supranol Orange RA (Acid Orange 45—C.I. 22195)      | 1               | 3   | 1     | 2   |               |   |
|    | Supranol Red RL (Acid Red 99—C.I. 23285)            | 3               | 4-5 | 2     | 4-5 | 5             | 6 |
|    | Supranol Red PG (Acid Red 85—C.I. 22245)            | 2               | 4   | 2     | 4   | 5             | 5 |
|    | Supranol Brilliant Red BA (Acid Red 133—C.I. 17995) | 2               | 3   | 1-2   | 3   |               |   |
| 75 | Supranol Red PBX (Acid Red 114—C.I. 23635)          | 2               | 3   | 1-2   | 2   |               |   |

| Employing dye bath                                                                        | Improvement in-- |     |       |     |               |       |
|-------------------------------------------------------------------------------------------|------------------|-----|-------|-----|---------------|-------|
|                                                                                           | Levelness        |     | Barré |     | Lightfastness |       |
|                                                                                           | A                | B   | A     | B   | A             | B     |
| Supra Light Rubine BLA<br>(Acid Red 32—C.I. 17065)                                        | 3                | 4-5 | 2     | 4-5 | 5             | 6     |
| Alizarine Sky Blue BS (Acid<br>(Blue 78—C.I. 62105)                                       | 4                | 4-5 | 3-4   | 4-5 | 6             | 6     |
| Alizarine Supra Sky RA (Acid<br>Blue 62—C.I. 62045)                                       | 3                | 4   | 2     | 4   | 5             | 6     |
| Alizarine Cyanine Green GHN<br>(Acid Green 25—C.I. 61590)                                 | 2                | 4   | 1     | 4-5 | 6             | 6     |
| Alizarine Cyanine Green GWA<br>(Acid Green 44—C.I. 61590)                                 | 3                | 4-5 | 3     | 4-5 | 6             | 6     |
| Sulphon Cyanine 5 RA (Acid<br>Blue 113—C.I. 26360)                                        | 1                | 3   | 1     | 3   | .....         | ..... |
| Sulphon Cyanine GRA (Acid<br>Blue 120—C.I. 26400)                                         | 1                | 1   | 1     | 2   | .....         | ..... |
| Sulphon Cyanine GA (Acid<br>Blue 118—C.I. 26410)                                          | 1                | 3   | 1     | 3   | .....         | ..... |
| Palatine Black WAN (Acid<br>Black 52—C.I. 15711)                                          | 2                | 2-3 | 1     | 2   | .....         | ..... |
| Supranol Red RA (Mixture of<br>C.I. Acid Red 114—C.I. 23635<br>and C.I. Acid Red 85-2245) | 2                | 3   | 1-2   | 2   | .....         | ..... |
| Supranol Brilliant Red 30 (Acid<br>Red 155—C.I. 18130)                                    | 1                | 4-5 | 2     | 4-5 | 3-4           | 3-4   |
| Supranol Blue GG (Acid Blue<br>127—C.I. 61135)                                            | 1                | 3-4 | 1     | 3   | .....         | ..... |
| Alizarine Green 5G (Acid<br>Green 4—C.I. 62560)                                           | 2                | 4-5 | 2     | 4   | 5-6           | 6     |

## EXAMPLE II

Comparative dyeings were made of 10 gram samples of taffeta (nontexturized nylon 66 filaments). The fabric was rolled and introduced in the stainless steel wire baskets available on the Vistamatic (Ahiba) automatic dyeing equipment. The dye baths comprised:

- 0.2 percent of Dye OWF
- 0.2 percent OWF Dye and 4 percent sodium bis(2,6-dimethyl-heptyl-4)sulfosuccinate.

The baths were established at a ratio of 1 gram of fabric to 40 cc. of liquid and the temperature raised to 200° F., over a period of 45 minutes. After the first 30 minutes at this temperature 1 percent of acetic acid (56 percent) was added to both (a) and (b). The dyeings were maintained at 200° F., for 30 minutes longer and the samples were subsequently rinsed and dried.

The dyeings were rated for levelness and barré as in example I. As may be seen from table II there was a dramatic improvement in both levelness and barré when sodium bis(2,6-dimethyl-heptyl-4)sulfosuccinate was employed in the dye bath.

30 35 40 45 50

TABLE II

|                                                                | Improvement in<br>Levelness |     |       |     |
|----------------------------------------------------------------|-----------------------------|-----|-------|-----|
|                                                                | (a)                         | (b) | Barré |     |
|                                                                | (a)                         | (b) |       |     |
| Milling Yellow O (Acid Yellow 38)<br>(C.I. 25135)              | 2                           | 5   | 3     | 5   |
| Wool Fast Orange GA (Mordant Orange<br>6)<br>(C.I. 26520)      | 2                           | 5   | 3     | 5   |
| Supranol Red PG Extra (Acid Red 85)<br>(C.I. 22245)            | 1                           | 2   | 4-5   | 4   |
| Supranol Red RL (Acid Red 99)<br>(C.I. 23285)                  | 2                           | 4-5 | 2     | 4-5 |
| Supranol Light Rubine BLA (Acid Red<br>32)<br>(C.I. 17065)     | 3                           | 5   | 3     | 4-5 |
| Alizarine Astrol B (Acid Blue 27)<br>(C.I. 61530)              | 2                           | 3   | 5     | 4-5 |
| Alizarine Sky Blue BS (Acid Blue 78)<br>(C.I. 62105)           | 3-4                         | 5   | 3-4   | 4-5 |
| Alizarine Supra Sky RA (Acid Blue 62)<br>(C.I. 62045)          | 4                           | 5   | 3-4   | 5   |
| Alizarine Cyanine Green GHN (Acid<br>Green 25)<br>(C.I. 61570) | 2                           | 4-5 | 2     | 4-5 |

## EXAMPLE III

Texturized nylon (nylon 66—Banlon, Joseph Bancroft & Company) was added at room temperature to three groups of dye baths, each comprising:

for Group 1: 0.2 percent Dye-OWF

The temperature of these dye baths were raised to 190° F., for 30 minutes. 10 percent common salt was then added and the dyeing continued at 190° F., for 45 additional minutes. The dyeings were then rinsed and dried.

for Group 2: 0.2 percent Dye-OWF

The dyeings in this group were handled exactly as in group 1 except for the temperature which was maintained at the boil.

for Group 3: 0.2 percent Dye-OWF

4.0 percent OWF Sodium bis(2,6-dimethyl-heptyl-4)sulfosuccinate. The temperature of these dye baths were raised to 190° F., and held at 190° F., for 30 minutes. 1 percent acetic acid (56 percent) was then added and the dye bath maintained at 190° F., for 30 minutes longer. The fabric was then rinsed and dried. Table III lists barré and lightfastness ratings for each group of dyeings according to the rules set forth in example I. As can be noted from table III, the use of the sulfosuccinate in the dye bath has resulted in practically barré free dyeings at temperatures considerably below the boil which also show a lightfastness superior to that of the dyeings in group 1 and 2. The dyes employed correspond to the following formulas.



VI



VII



VIII



5

10

15

20

## EXAMPLE V

Comparative dyeings were made of 10 g. samples of tiger cloth (i.e., a knit fabric made of alternating bands of variously textured filament nylon 66) added to a dye bath comprising: 0.2 percent dye OWF

which was then raised over a period of 30 minutes to the boil. Ten percent common salt was then added and the dye bath temperature maintained for an additional 45 minutes. As may be seen from table V, the dyeings had a predominant barre effect.

## EXAMPLE VI

Ten gram samples of tiger cloth were added to a dye bath comprising 0.2 percent Dye and 4 percent Sodium bis-(2,6-dimethyl-heptyl-4) sulfosuccinate. The temperature of this dye bath was raised to the boil over a period of 30 minutes and 1 percent acetic acid was then added. The temperature of the dye bath was maintained for an additional 45 minutes. As may be seen from table V, the resulting dyeings were free from the barre effect.

TABLE III

| Dye (corresponding to structure number) | Percent | Group I |               | Group II |               | Group III |               |
|-----------------------------------------|---------|---------|---------------|----------|---------------|-----------|---------------|
|                                         |         | Barre   | Lightfastness | Barre    | Lightfastness | Barre     | Lightfastness |
| I                                       | 0.2     | 3       | 4             | 3        | 4             | 4         | 5             |
| II                                      | 0.2     | 4       | 4             | 4        | 4             | 4-5       | 4-5           |
| III                                     | 0.2     | 4       | 5             | 4        | 5             | 4-5       | 5             |
| IV                                      | 0.2     | 4       | 5             | 4        | 5-6           | 4-5       | 6             |
| V                                       | 0.2     | 3       | 5-6           | 3-4      | 5-6           | 4         | 6             |
| VI                                      | 0.2     | 3       | 4             | 3-4      | 5             | 4         | 5-6           |
| VII                                     | 0.2     | 4       | 6             | 4        | 5-6           | 4-5       | 6             |
| VIII                                    | 0.2     | 2-3     | 5-6           | 3        | 5-6           | 4         | 6-7           |
| Alizarine Supra Blue A                  | 0.2     | 4       | 4             | 4        | 4-5           | 4         | 4-5           |

## EXAMPLE IV

Texturized nylon (nylon 66 - Banlon, Joseph Bancroft & Company) was added at room temperature to three groups of dye baths prepared and handled exactly as in example III for the use of 0.5 percent OWF of dye in each.

Table IV in addition to listing barre and lightfastness ratings for each group of dyeings according to the rules set forth in example I, also gives ratings for the degree of dye exhaustion.

The degree of exhaustion rating was obtained in the following manner.

After the dyeings were removed the dye baths were strongly acidified by the addition of 2 percent OWF of formic acid (90 percent). Undyed nylon 66 skeins of equal weight to the samples dyed were immersed in the bath so prepared and run at the boil for 45 minutes. After rinsing and drying these skeins the depth of dyeing was compared to that of the original dyeings estimating in this fashion the percent of dye removed from the dye bath by the original dyeing.

Table IV confirms the results observed in example III and in addition, shows that the use of the sulfosuccinate followed by lowering of the pH of the dye bath has resulted in as good a degree of exhaustion of the dyestuff from the baths as that obtained in the dyeings without additive (group 1 and 2).

## TABLE V

| Dye<br>(Same as<br>Table III) | Barre | 10% Salt after<br>First 30 min. | 4% Sodium bis-(2,6-<br>dimethyl-heptyl-4)<br>sulfosuccinate | 1% Acetic acid<br>after first 30 min. |         |          |
|-------------------------------|-------|---------------------------------|-------------------------------------------------------------|---------------------------------------|---------|----------|
|                               |       |                                 |                                                             |                                       | (Ex. V) | (Ex. VI) |
| I                             | 3     |                                 |                                                             |                                       | 5       |          |
| II                            | 4     |                                 |                                                             |                                       | 5       |          |
| III                           | 2-3   |                                 |                                                             |                                       | 3       |          |
| IV                            | 4     |                                 |                                                             |                                       | 5       |          |
| V                             | 3     |                                 |                                                             |                                       | 4       |          |
| VI                            | 3     |                                 |                                                             |                                       | 4       |          |
| VII                           | 3     |                                 |                                                             |                                       | 4-5     |          |
| VIII                          | 2-3   |                                 |                                                             |                                       | 4       |          |
| Alizarine Supra<br>Blue A     | 3-4   |                                 |                                                             |                                       | 5       |          |

## EXAMPLE VII

Twenty gram samples of nylon 6 carpet (Allied Chemical Corporation) were dyed in dye baths comprising:  
a. 0.2 percent OWF Celliton Fast Blue FFRN (Disperse

TABLE IV

| Dye                    | Per-<br>cent | Group 1 |                    | Group 2                            |       | Group 3            |                                    |       |                    |                                    |
|------------------------|--------------|---------|--------------------|------------------------------------|-------|--------------------|------------------------------------|-------|--------------------|------------------------------------|
|                        |              | Barre   | Light-<br>fastness | Estimated<br>percent<br>exhaustion | Barre | Light-<br>fastness | Estimated<br>percent<br>exhaustion | Barre | Light-<br>fastness | Estimated<br>percent<br>exhaustion |
| I                      | 0.5          | 3-4     | 5-6                | 60                                 | 3-4   | 5-6                | 60                                 | 4-5   | 6                  | 60                                 |
| II                     | 0.5          | 4       | 5-6                | 98                                 | 4     | 5-6                | 95                                 | 4-5   | 6                  | 98                                 |
| III                    | 0.5          | 4-5     | 6                  | 90                                 | 4-5   | 6                  | 85                                 | 5     | 6                  | 95                                 |
| IV                     | 0.5          | 4       | 6                  | 98                                 | 4     | 7                  | 95                                 | 4-5   | 6-7                | 98                                 |
| V                      | 0.5          | 3       | 6                  | 98                                 | 3-4   | 6                  | 95                                 | 4     | 6                  | 98                                 |
| VI                     | 0.5          | 3       | 5-6                | 98                                 | 3-4   | 6                  | 98                                 | 4     | 6                  | 98                                 |
| VII                    | 0.5          | 4       | 6-7                | 95                                 | 4     | 6                  | 90                                 | 4-5   | 6                  | 95                                 |
| VIII                   | 0.5          | 3       | 6                  | 98                                 | 3     | 6                  | 95                                 | 4     | 7                  | 98                                 |
| Alizarine Supra Blue A | 0.5          | 4       | 5-6                | 90                                 | 4     | 5-6                | 80                                 | 4-5   | 6                  | 90                                 |

Blue 3-C.I. No. 61505); 4 percent OWF Sodium bis-(2,6-dimethyl-heptyl-4) sulfosuccinate

b. 0.2 percent OWF Celliton Fast Blue FFRN (Disperse Blue 3-C.I. No. 61505). The ratio of carpet to water was 1 gram of carpet to 40 ccs. of water. The temperature of both baths was raised to the boil in 45 minutes and maintained there for a period of 1 hour. The samples were rinsed and water extracted in a centrifuge and the samples subsequently dried. The nylon sample from bath (a) showed a brilliant blue shade, while the sample from bath (b) was considerably greener and duller. The samples were subsequently exposed to the (Fade-o-Meter) carbon arc light source for 20 hours and sample (a) exhibited little fading, while sample (b) demonstrated a dramatic loss to yellow-green cast.

#### EXAMPLE VIII

Samples of nylon 6 carpet (Allied Chemical Corporation) were dyed in dye baths having the following composition:

- a. 0.2 percent Supra Light Rubine BLA (Acid Red 32-C.I. No. 17065)
- b. 0.2 percent Supra Light Rubine BLA 4 percent Sodium bis-(2,6-dimethyl-heptyl-4) sulfosuccinate
- c. 0.2 percent Alizarine Fast Gray BLN (Acid Black 48-C.I. No. 65005)
- d. 0.2 percent Alizarine Fast Gray BLN 4 percent Sodium bis-(2,6-dimethyl-heptyl-4) sulfosuccinate.

All the dye baths were raised to the boil over a period of 45 minutes. After the first 30 minutes 1 percent acetic acid (56 percent) was added to each of the dye baths to complete the exhaustion of the dyes from the bath. Sample (a) showed an uneven dyeing result due to barre and not to a lack of levelness, and the color was altered by lignin to a brick red color. Sample (b) showed an improved dyeing result and the barre effect was greatly reduced and the true shade of the Rubine dye was unaltered by lignin. Sample (c) resulted in an uneven dyeing due to barre and a greenish-gray shade of color, while sample (d) showed a much more uniform dyeing and a considerable reduction in barre and the true blue shade characteristic of the dye was apparent.

#### EXAMPLE IX

Comparative dyeings were made of 10 gram samples of nylon 66, nylon 6, nylon 11, nylon 610, nylon 66/6, Perlon and Rilsan, using dyes particularly comprising those in table I:

- a. 0.2 percent OWF Dye plug 1 percent ethoxylated nonionic surfactant comprising nonyl phenol + 30 mols E.O., 75 percent active and 6 percent ammonium sulfate.
- b. 0.2 percent OWF Dye plus 4 percent Sodium bis-(2,6-dimethyl-heptyl-4) sulfosuccinate.

In each instance there was a dramatic improvement both in levelness and barre effect when sodium bis-(2,6-dimethyl-heptyl-4) sulfosuccinate was employed in the dye bath, as per the procedure in example I.

#### EXAMPLE X

Comparative dyeings were made of 10 gram samples of textured nylon 66 using dye baths comprising those in table I:

- a. 0.2 percent OWF Dye plus 1 percent ethoxylated nonionic surfactant comprising nylon phenol + 30 mols E.O., 75 percent active and 6 percent ammonium sulfate.
- b. 0.2 percent OWF Dye plus 4 percent Sodium bis-(2,6-dimethyl-heptyl-4) sulfosuccinate.

#### EXAMPLE XI

The procedure of examples IX and X were repeated except that the particular sulfosuccinates employed were bis(1,4-diethyl-heptyl) sulfosuccinate, bis(1,3-diisopropyl butyl) sulfosuccinate, bis(3,5-dimethyl-octyl-5) sulfosuccinate, bis(1,7-diethyl tetradecyl-10) sulfosuccinate, bis(1,3-dimethyl butyl-1) sulfosuccinate, bis(3,8-butyl heptyl-5) sulfosuccinate, and bis(1,7-diphenyl octyl-4) sulfosuccinate, etc. In each instance there was a dramatic improvement in both levelness and barre effect when the sulfosuccinate was employed as compared to the process when said sulfosuccinate was not employed.

In the preceding examples the term "nylon" relates to the polyamide fiber obtained by condensing adipic acid with hexamethylenediamine, "nylon 610" denotes the polyamide fiber obtained by condensing sebacic acid with hexamethylenediamine, "nylon 66/6" is the polyamide copolymer obtained by condensing together adipic acid, hexamethylenediamine and caprolactam, "Perlon" is the polyamide fiber obtained from caprolactam and "Rilsan" that obtained from waminoundecylic acid.

Furthermore, in the preceding examples and throughout the specification, all indicated percentages are based on the weight of the fibrous goods employed as indicated by OWF.

As noted in the above examples and throughout the specification there may be added an acid such as acetic acid toward the end of the dyeing process to complete the exhaustion of the dyestuffs. Furthermore, as previously noted the acidification may also be employed for similar purposes wherein barre dyeings are repaired by subsequent treatment. Preferably, acetic acid is employed in those processes which require acidification. In addition, however, other organic or inorganic acids can also be employed in the known manner, such acids including formic acid, acetic acid, hydrochloric acid, sulfuric acid, phosphoric, alkyl and aryl sulfonic acids, and their acidic salts such as ammonium sulfate and the like.

In addition, as previously noted some of the dyeing processes are operative after an initial treatment with alkalizing materials. Those alkalizing materials which may be employed include but are not limited to ammonium hydroxide and alkali metal salts of weak acids such as sodium acetate and the like.

What is claimed is:

- 1. A method of producing improved polycarbonamide fibrous dyeings consisting essentially of treating polycarbonamide fibrous material with an aqueous medium comprising from 0.1-10 percent by weight based on the weight of the fibrous material of a water-soluble salt of a dialkyl sulfosuccinate containing from about 12 to about 40 carbon atoms, in the presence of an acid dye.
- 2. The method of claim 1 wherein the dialkyl sulfosuccinate is a bis-nonyl sulfosuccinate.
- 3. The method of claim 1 wherein the salt of a dialkyl sulfosuccinate is sodium bis-(2,6-dimethyl-heptyl-4) sulfosuccinate.
- 4. The process of claim 1 wherein the pH of the dye bath is about 3 to about 7.
- 5. The process of claim 2 wherein the pH of the dye bath is about 3 to about 7.
- 6. The process of claim 3 wherein the pH of the dye bath is about 3 to about 7.